

# UNITED STATES PATENT OFFICE.

FRANCIS M. McCLENAHAN, OF OAKMONT, PENNSYLVANIA.

## PROCESS OF RECOVERING METALS FROM SILICATES.

1,426,891.

Specification of Letters Patent. Patented Aug. 22, 1922.

No Drawing.

Application filed December 7, 1921. Serial No. 520,601.

To all whom it may concern:

Be it known that I, FRANCIS M. McCLENAHAN, a citizen of the United States, and a resident of Oakmont, in the county of Allegheny and State of Pennsylvania, have invented a new and useful Improvement in Processes of Recovering Metals from Silicates, of which the following is a specification.

10 The invention relates to the recovery of metals, particularly aluminum and potassium, from silicates containing them, and has particularly to do with the breaking up of double ammonium-aluminum fluorides formed in the process of recovering from aluminous silicates such as kaolin, feldspar, leucite, glauconite, etc., metals whose silico-fluoride or whose hydroxides are practically insoluble in an aqueous solution of ammonium fluorides and ammonium hydroxide, which process is disclosed in my pending application Serial No. 432,518, filed December 22, 1920.

According to the process disclosed in said application and contemplated herein, ground or otherwise pulverized silicates of aluminum to which water is preferably added to form a pasty or semi-fluid mixture, is decomposed by the addition of a fluoride of ammonium in excess of that theoretically required to reduce the constituent elements to an aqueous solution of fluo-silicates containing hydrated oxide of aluminum as a precipitate. This decomposition is effected 35 preferably at about the boiling temperature of the mixture. While the fluoride of ammonium may be neutral, basic or acid, it is preferred to use acid ammonium fluoride, commercially known as ammonium bi-fluoride. The silicates require no treatment previous to their being mixed with the fluoride of ammonium, it being only necessary from a practical standpoint that they be sufficiently pulverized to permit them to be freely 40 and rapidly decomposed.

When feldspar is so decomposed the reaction may in part be expressed by the following equation:



In addition to this reaction it has been 55 found that a series of chemical reactions take place giving rise to the presence of double ammonium-aluminum fluorides such as

$AlF_3 \cdot 3NH_4F$ , the tenacity of the union of which is very pronounced. The following equation expresses the chemical reaction 60 which may take place incident to the formation of such double ammonium-aluminum fluorides.



The double ammonium-aluminum fluoride is formed by a portion of the ammonium 70 fluoride ( $NH_4F$ ) of the right hand portion of the equation uniting with the aluminum fluoride ( $AlF_3$ ).

The object of the present invention is to improve the process thus explained to the end 75 that the tenacious double ammonium-aluminum fluorides may be broken up readily and aluminum recovered as a hydrated oxide and potassium as a silico-fluoride. A further object is to provide an improved process of hydrolyzing double ammonium-aluminum fluorides regardless of how they may be formed. 80

In the practice of this invention the precipitate of equations 1 and 2 is heated in the presence of water to a temperature sufficient 85 high to cause the aluminum fluoride of the double ammonium-aluminum fluorides to decompose. This decomposition is attended by the formation of hydrated aluminum oxide and hydrofluoric acid, the latter of which 90 unites with the ammonium fluoride of the original double ammonium-aluminum fluorides to form ammonium bi-fluoride, which, at the temperature of the reaction is vapor. To prevent the ammonium bi-fluoride vapor 95 from reacting with the hydrated aluminum oxide it is continuously removed from the receptacle in which the double ammonium-aluminum fluorides are treated. The reaction which takes place in this treatment may 100 be expressed by the following equation:



Before the precipitate resulting from the 105 reactions of equations 1 and 2 is treated in the manner described, it may, if desired be washed in hot water to remove the ammonium silico-fluoride which ordinarily adheres quite closely to the sludge, and the resulting 110 sludge and liquor may be separated in a settling tank. While the moist sludge may then be placed in a retort and heated either indirectly by external heat or directly by passing

hot air or steam through it to hydrolyze the double ammonium-aluminum fluorides, the sludge is preferably first dried and then heated in a suitable retort by passing superheated steam through it, the steam being at a temperature of not less than about 300° C. For rapidity of action the temperature of the steam may be as high as 400° C.

By thus injecting heated steam into the dried mass, the steam serves five purposes,— it heats the mass to the temperature required to decompose the aluminum fluoride, it furnishes water for the oxidation and hydrating of the aluminum, it vaporizes such potassium silico-fluorides as may be present in the mass, it agitates the mass, and it removes the liberated vapors from the mass and the retort. By agitating the mass and removing the liberated hydrofluoric acid and ammonium fluoride vapors, the steam prevents subsequent reaction of these vapors upon the hydrated aluminum oxide.

The liberated and removed vapors may be subsequently condensed, preferably by passing them into water. The hydrofluoric acid and ammonium fluoride combine to form water soluble ammonium bi-fluoride, while the water insoluble potassium silico-fluoride forms a sludge which may easily be separated from the aqueous condensate. In case the ammonium silicofluoride is not washed or otherwise removed from the precipitate of equations 1 and 2, it too will pass off as a vapor from the mass when heated in the manner described, and subsequently may be condensed and separated from the condensed ammonium bi-fluoride.

At the completion of the heating operation the treated mass is hydrated aluminum oxide, with which there may be mixed small quantities of impurities such as mica, free silica, iron oxide, etc., which may be present in the silicates originally digested. The filtrate of equations 1 and 2 may be treated in the manner disclosed in my above identified application.

While the invention has been explained chiefly with reference to its applicability to the recovery of alumina from silicates containing them, it is also applicable to the recovery of hydrated oxide of aluminum from double ammonium-aluminum fluorides regardless of whether they are formed in the digesting of silicates by a fluoride of ammonium.

I claim as my invention:

1. The process of recovering metals from silicates containing them, which comprises decomposing the silicates by a fluoride of ammonium, separating the resulting precipitate from the liquor, and simultaneously heating the precipitate in the presence of water and removing and condensing the resulting vapors.

65 2. The process of recovering alumina

from silicates containing them, which comprises decomposing the silicates by a fluoride of ammonium, separating the resulting precipitate from the liquor, and simultaneously agitating the precipitate, heating it to a temperature of not less than about 300° C., and removing the resulting vapors, whereby hydrated oxide of aluminum is formed.

3. The process of recovering alumina from silicates containing them, which comprises decomposing the silicates by a fluoride of ammonium, separating the resulting precipitate from the liquor, and simultaneously injecting into the precipitate steam heated to a temperature of not less than about 300° C. and removing the resulting vapors, whereby hydrated oxide of aluminum is formed.

4. The process of recovering metals from silicates containing them, which comprises decomposing the silicates by an excess of ammonium bi-fluoride in the presence of water, separating the resulting precipitate from the liquor, drying the precipitate, and simultaneously passing through the dried precipitate steam heated to a temperature of not less than about 300° C., and removing the resulting vapors.

5. The process of recovering hydrated oxide of aluminum from an intimate mixture of aluminum and ammonium fluorides, which comprises heating said mixture in the presence of water and simultaneously removing the resulting vapors.

6. The process of recovering hydrated oxide of aluminum from an intimate mixture of aluminum and ammonium fluorides, which comprises simultaneously agitating and heating the mixture and removing the resulting vapors.

7. The process of recovering hydrated oxide of aluminum from an intimate mixture of aluminum and ammonium fluorides, which comprises simultaneously heating the mixture to a temperature of not less than about 300° C., agitating it and removing the resulting vapors.

8. The process of recovering hydrated oxide of aluminum from an intimate mixture of aluminum and ammonium fluorides, which comprises passing through said mixture steam heated to a temperature of not less than about 300° C., and simultaneously removing the resulting vapors.

9. The process of hydrolyzing double ammonium-aluminum fluorides which comprises passing through them steam heated to not less than about 300° C., and simultaneously removing in vapor form the resulting ammonium bi-fluoride.

In testimony whereof, I sign my name.  
FRANCIS M. McCLENAHAN.

Witnesses:

EDWIN O. JOHNS,  
PAUL N. CRITCHLOW.